

E. A. C. SMITH.

ELECTRODE.

APPLICATION FILED JAN. 7, 1918.

1,311,096.

Patented July 22, 1919.

Fig. 1,



Fig. 2,



Fig. 3,



Fig. 4,



Fig. 5.



E. A. C. Smith INVENTOR

BY  
Perry Davis Marvin & Edwards  
ATTORNEYS

# UNITED STATES PATENT OFFICE.

ELIAS ANTHON CAPPELEN SMITH, OF NEW YORK, N. Y.

## ELECTRODE.

1,311,096.

Specification of Letters Patent. Patented July 22, 1919.

Application filed January 7, 1918. Serial No. 210,740.

To all whom it may concern:

Be it known that I, ELIAS ANTHON CAPPELEN SMITH, a citizen of the United States, residing at No. 440 Riverside Drive, in the 5 county of New York, State of New York, have invented certain new and useful Improvements in Electrodes; and I do hereby declare the following to be a full, clear, and exact description of the invention, such as 10 will enable others skilled in the art to which it appertains to make and use the same.

The electrolytic deposition of metals, such as copper, from acid solutions, such as sulfate solutions, requires, for its successful 15 practice, that the anodes utilized shall be resistant to the acid liquor of the electrolyte and to the corroding effect of the electrolytic operation; and, also, that the anode itself shall not, because of such solution or 20 corrosion, contaminate the electrolyte to the prejudice of the electrolytic deposition.

When the electro-deposition takes place from electrolytes containing oxidizing 25 agents, such as nitric acid or chlorin or ferric sulfate, the anodes are required to have a correspondingly increased resistance to 30 corrosion thereby. Anodes of lead or antimonial lead, such as are commonly used in electro-deposition from acid electrolytes, and 35 which are resistant to corrosion in the absence of such oxidizing agents, are rapidly corroded when such oxidizing agents are present, with a resulting short life of the anodes and contamination of the electrolyte.

35 The present invention is based on the discovery that anodes of silicon iron, of proper silicon content, are resistant, not only to acid electrolytes, but also to corrosion, when used as anodes for electro-deposition from 40 acid electrolytes, even where the electrolyte contains appreciable amounts of oxidizing agents, such as nitric acid and chlorin.

The silicon iron utilized in the production of the anodes of the present invention may 45 contain, for example, 14 to 15% of silicon, although the proportions are capable of some variation, *e. g.*, between 12 and 20 per cent. If the silicon content becomes too low, the anodes become less resistant; while 50 if the silicon content becomes too high, the anodes become brittle and the voltage becomes excessive. The silicon iron may contain not only silicon and iron, but it may contain other ingredients provided they are 55 not prejudicial to the resistivity of the anode to electrolytic anodic corrosion.

Silicon iron of the composition referred to is hard, and difficult to work or machine. If the anodes made therefrom are provided with detachable clamps for leads, an excessive amount of current is lost due to the drop in voltage at the clamp. I have found, however, that the silicon iron, although of high melting point, can nevertheless be provided with conductive leads, for example, 60 of copper, when the anodes are produced by a casting operation; and that an integral union between the copper lead and the silicon iron of the anode can be thus produced. As the result of this construction, the drop 65 in voltage and accompanying loss in power at the contacts or leads can be very materially reduced, so that the electrodes are well adapted for use for commercial purposes, without excessive power consumption. 70

The silicon iron anodes of the present invention, with the copper leads cast therein, may be, for example, of a size of about four feet in length,  $4\frac{1}{2}$  inches wide, and one inch thick, with two copper leads of about one-quarter inch in diameter cast therein at one 75 end.

The anodes may thus be cast in a sand mold with the copper leads arranged in the bottom of the mold and with chill plates at 80 the bottom of the mold to chill that portion of the anode adjacent to the leads and thereby prevent melting of the copper. The melting point of the copper conductive leads is lower than the melting point of the silicon iron, and the rapid cooling and consequent solidification of the portions of the molten silicon iron in contact with and adjacent to the conductive leads, as a result of 85 the use of chill plates, prevents the melting 90 of the metal of the conductive leads during 95 the casting operation.

The conductive leads are thus embedded in the cast silicon iron anode and, while in 100 intimate mechanical and electrical contact therewith, are physically separate and distinct therefrom.

An anode illustrative of the present invention is shown in the accompanying drawings, in which Figure 1 shows a series of 105 five anodes spaced apart as in an instance of actual operation. Fig. 2 is a side view of one of the anodes; Fig. 3 is a top view of the anodes of Fig. 1; and Figs. 4 and 5 are respectively side and edge detail views of one 110 of the copper leads.

In Fig. 1 a series of anodes 1, 2, 3, 4 and

5 is shown arranged as they are supported from a suitable support (not shown) during the electrolytic operation. Each of the anodes is provided with two copper contacts 5 6 cast therein, these contacts having one end 7 embedded and cast in the anode and the other end 8 flattened and provided with a hole 9 for connection with the current and with the support.

10 The anodes at their lower ends may be provided with holes 10 which may be made therein during the casting operation; and a fiber or wooden bar 11 may be arranged in these holes for assisting in keeping the 15 anodes properly spaced apart and in alignment when used.

With the anodes of the present invention, it is possible to distribute the current evenly to the electrolyte, with the avoidance of excessive losses such as would be involved with anodes having poor contacts, and with a minimum corrosion of the anodes during the electrolysis.

The resistance of the anodes of the present invention to corrosion, when used as 25 anodes, is such that they may be used for considerable periods of time, for example, as anodes in the electrolytic decomposition of copper from sulfate solutions, even where

the solutions contain appreciable amounts of 30 nitric acid or chlorin.

I claim:

1. An electrode composed of cast silicon iron having a conductive lead of a metal of lower melting point than said silicon iron, 35 one end of said conductive lead being embedded in the solid silicon iron and in intimate mechanical and electrical contact therewith while physically separate and distinct therefrom; substantially as described. 40

2. An electrode composed of silicon iron having partially embedded therein a conductive lead of copper, said conductive lead being in intimate mechanical and electrical contact with said silicon iron while physically separate and distinct therefrom: substantially as described. 45

3. An electrode of silicon iron having partially embedded therein one or more conductive leads of a metal of lower melting point than said silicon iron, said conductive lead or leads being in intimate mechanical and electrical contact with said silicon iron while physically separate and distinct therefrom; substantially as described. 50

In testimony whereof I affix my signature.

ELIAS ANTHON CAPPELEN SMITH.